# EUROPEAN PATENT SPECIFICATION

(11) **EP 0 342 921 B1**
(45) Date of publication and mention of the grant of the patent: **01.09.1993**
(21) Application number: 89304925.4
(22) Date of filing: 16.05.1989
(51) Int. Cl.: H01F 1/14, C22C 38/16, C21D 6/00

(54) **Fe-based soft magnetic alloy**
Weichmagnetische Legierung auf Eisenbasis
Alliage magnétique mou à base de fer

(30) Priority: 17.05.1988 JP 118331/88
(43) Date of publication of application: 23.11.1989
(73) Proprietor: KABUSHIKI KAISHA TOSHIBA, Kawasaki-shi, Kanagawa-ken 210 (JP)
(72) Inventor: Sawa, Takao c/o Intellectual Property Division, Tokyo (JP); Okamura, Masami c/o Intellectual Property Division, Tokyo (JP)
(74) Representative: BATCHELLOR, KIRK & CO.

(56) References cited:
- EP-A- 0 271 657
- EP-A- 0 302 355
- CH-A- 443 505
- DE-B- 2 005 371
- JP-A- 4 992 600
- JP-A- 5 273 120
- JP-A- 5 449 936

## Description

This invention relates to Fe-based, soft magnetic alloys.

Conventionally, iron cores of crystalline materials such as permalloy or ferrite have been employed in high frequency devices such as switching regulators. However, the resistivity of permalloy is low, so it is subject to large core loss at high frequency. Also, although the core loss of ferrite at high frequencies is small, the magnetic flux density is also small, at best 5,000 G. Consequently, in use at high operating magnetic flux densities, ferrite becomes close to saturation and as a result the core loss is increased.

Recently, it has becomes desirable to reduce the size of transformers that are used at high frequency, such as the power transformers employed in switching regulators, smoothing choke coils, and common mode choke coils. However, when the size is reduced, the operating magnetic flux density must be increased, so the increase in core loss of the ferrite becomes a serious practical problem.

For this reason, amorphous magnetic alloys, i.e., alloys without a crystal structure, have recently attracted attention and have to some extent been used because they have excellent soft magnetic properties such as high permeability and low coercive force. Such amorphous magnetic alloys are typically base alloys of Fe, Co, Ni, etc., and contain metalloids as elements promoting the amorphous state, (P, C, B, Si, Al, and Ge, etc.).

However, not all of these amorphous magnetic alloys have low core loss in the high frequency region. Iron-based amorphous alloys are cheap and have extremely small core loss, about one quarter that of silicon steel, in the frequency region of 50 to 60 Hz. However, they are extremely unsuitable for use in the high frequency region for such applications as in switching regulators, because they have an extremely large core loss in the high frequency region of 10 to 50 kHz. In order to overcome this disadvantage, attempts have been made to lower the magnetostriction, lower the core loss, and increase the permeability by replacing some of the Fe with non-magnetic metals such as Nb; Mo, or Cr. However, the deterioration of magnetic properties due to hardening, shrinkage, etc., of resin, for example, on resin molding, is large compared to Co-based alloys, so satisfactory performance of such of such materials is not obtained when used in the high frequency region.

Co-based, amorphous alloys also have been used in magnetic components for electronic devices such as saturable reactors, since they have low core loss and high squareness ratio in the high frequency region. However, the cost of Co-based alloys is comparatively high making such materials uneconomical.

As explained above, although Fe-based amorphous alloys constitute cheap soft magnetic materials and have comparatively large magnetostriction, they suffer from various problems when used in the high frequency region and are inferior to Co-based amorphous alloys in respect of both core loss and permeability. On the other hand, although Co-based amorphous alloys have excellent magnetic properties, they are not industrially practical due to the high cost of such materials.

### Summary of the Invention

Consequently, having regard to the above problems, the object of this invention is to provide an Fe-based, soft magnetic alloy having high saturation magnetic flux density in the high frequency region and with excellent soft magnetic characteristics.

According to the invention, there is provided an Fe-based soft magnetic alloy having fine crystal grains, as described in the following formula (I)

Fe_{100-a-b-c-d}MₐM'_{b}Z_{c}N_{d} (I)

where M is at least one element from the following: Cu, Ag, Au, Zn, Sn, Pb, Sb, and Bi;
M' is at least one element from the following: Ti, Zr, Hf, V, Nb, Ta, Cr, Mo, W, or Mn, Co, Ni, and Al;
Z is at least one element from the following: Si, P, and B;
and wherein a, b, c and d, expressed in atomic % are as follows:
0.01 ≦ a ≦ 5
0.1 ≦ b ≦ 10
15 ≦ c ≦ 28
0 < d ≦ 8.

Fine crystal grains are present in the alloy to the extent of 30%, in the range of 5 to 30 nm (50 to 300 Å) or more in terms of area ratio. At least 80% of the fine crystal grains should be of a crystal grain size of 5 to 30 nm (50 Å to 300 Å). The term "area ratio" of the fine crystal grains as used herein means the ratio of the surface of the fine grains to the total surface in a plane of the alloy as measured, for example, by photomicrograph or by microscopic examination of ground and polished specimens.

In order that the invention may be illustrated and readily carried into effect, non-limiting preferred embodiments thereof will not be described by way of example only, with reference to the accompanying drawing wherein:
Fig. 1 is a graph showing the variation in core loss with variation of heat treatment temperature of alloy of the invention and of the alloy of a comparative example.

In order to obtain the desired composition of an alloy according to the invention, the composition thereof should be balanced and within the limits as hereinafter discussed.

An alloy in accordance with the invention contains: Fe; N; at least one of Cu, Ag, Au, Zn, Pb, Sb, and Bi; at least one of element from the group Ti, Zr, Hf, V, Nb, Ta, Cr, Mo, W, Mn, Co, Ni, and Al; and at least one of Si, P, and B; in accordance with the formula (I) as defined above.

It is important that alloys according to the invention contain the aforesaid components in the specified amounts to obtain the advantageous characteristics of the new alloys.

M is at least one of: Cu, Ag, Au, Zn, Sn, Pb, Sb and Bi.
These elements can be effective in increasing corrosion resistance, preventing coarsening of the crystal grains, and in improving soft magnetic properties such as core loss and permeability. However, if there is too little, the benefit of its addition is not obtained. On the other hand, if there is too much M, deterioration of magnetic properties results. A range of 0.01 to 5 atomic % is therefore selected. Preferably the amount is 0.5 to 3 atomic %.

M' is an element which can be effective in making the crystal grain size uniform and in improving the soft magnetic properties by reducing magnetostriction and magnetic anisotropy. It can also be effective in improving the magnetic properties in respect of temperature change. However, if the amount of M' is too small, the benefit of the addition is not obtained. On the other hand, if the amount is too large, the saturation magnetic flux density is lowered. An amount of M' in the range of 0.1 to 10 atomic % is therefore selected. Preferably the amount is 1 to 7 atomic % and even more preferably 1.5 to 5 atomic %.

In addition to the above-mentioned effects, the various additive elements in M' can have the following respective effects: in the case of Japanese Group IVa elements namely Ti, Zr and Hf, increase of the range of heat treatment conditions for obtaining optimum magnetic properties; in the case of Japanese Group Va elements namely V, Nb and Ta, and Mn, increase in resistance to embrittlement and increase in workability such as by cutting; in the case of Japanese Group VIa elements, namely Cr, Mo and W improvement of corrosion resistance and surface shape; in the case of A1, increased fineness of the crystal grains and reduction of magnetic anisotropy, thereby improving magnetostriction and soft magnetic properties.

Z comprises elements that can be effective in making the alloy amorphous during manufacture, or in directly segregating fine crystals. If the amount is too small, the benefit of superquenching in manufacture is difficult to obtain and the above condition is not obtained. On the other hand, if the amount of "Z" is too great, the saturation magnetic flux density becomes low, also making the above condition difficult to obtain, with the result that superior magnetic properties are not obtained. An amount in the range 15 to 28 atomic % is therefore selected. Preferably the range is 18 to 26 atomic %. In particular, the ratio of Si/B and/or Si/P is preferably more than 1.

Nitrogen is included because it can be effective in expanding the range of heat treatment conditions in order to obtain optimum magnetic properties. However, if there is too much N, fine crystals are difficult to obtain, so the amount is specified as being less than 8 at. %. Preferably it is less than 6 atomic %, and even more preferably less than 4 atomic %.

The Fe-based soft magnetic alloy of this invention may be obtained by the following method:
An amorphous alloy thin strip is obtained by liquid quenching, then heat treated for one minute to ten hours, preferably ten minutes to five hours at a temperature of 50C^{o} below to 120C^{o} above the crystallization temperature of the amorphous alloy, preferably 30C^{o} below to 100C^{o} above, to segregate the required fine crystals. Alternatively, direct segregation of the fine crystals can be accomplished by controlling quenching rate in the liquid quenching method.

It has also been determined that if there are insufficient fine crystal grains in the alloy of this invention, i.e., if there is too much amorphous phase, the core loss tends to become large, the permeability becomes low, the magnetostriction becomes large, and there is increased deterioration of the magnetic properties due to the resin moulding. It is thus preferable that there should be at least 30%, in terms of area ratio, of fine crystal grains in the alloy. More preferably, there should be at least 40%, and still more preferably at least 50%. Furthermore, it has been determined that if the size of the fine crystal grains is too small, the maximum improvement in magnetic properties is not obtained, while if it is too large, the magnetic properties are adversely affected. Consequently, it is desirable that at least 80% of the fine crystal grains should consist of crystals of crystal grain size 50 Å to 300 Å.

Fe-based soft magnetic alloys of this invention can have excellent soft magnetic properties at high frequency. They may exhibit excellent properties as an alloy for magnetic materials for magnetic components such as magnetic cores used at radio frequency, such as, for example, magnetic heads, thin film heads, radio frequency transformers including transformers for high power use, saturable reactors, common mode choke coils, normal mode choke coils, high voltage pulse noise filters, and magnetic switches used in laser power sources, and the like, and for sensors of various types, such as power source sensors, directions sensors, and security sensors, and the like.

### Examples

An amorphous alloy thin strip of thickness 15 µm was obtained by the single roll method from an alloy consisting of Fe₇₄Cu₂Mo₂Si₁₁B₉N₂. This amorphous alloy was then wound to form a toroidal core of external diameter 18 mm, internal diameter 12 mm, and height 4.5 mm, then heat treated for about 90 minutes at about 550°C. The crystallization of this alloy was about 575°C at a temperature rise rate of 10C^{o}/min (measured with a rate of temperature rise of 10C^{o}/min.

Fine crystal grains were present to the extent of about 85% with respect to the total area of the alloy in the magnetic core that was obtained. Of these, fine crystal grains of 50 Å to 300 Å represented about 90%.

Also, for comparison, a magnetic core was manufactured on which heat treatment was performed for about 40 minutes at about 450°C. It was found by TEM observation that fine crystal grains had not segregated in this magnetic core.

Comparing five samples of magnetic cores according to the invention in which fine crystal grains were present and five samples of the magnetic cores of the comparison sample in which fine crystal grains were not present, the core loss after heat treatment at 100 kHz, 2 kG and the core loss after epoxy coating, the magnetostriction, the permeability at 1 kHz 2 mOe, and the saturation magnetic flux density were measured. The mean values in each case are shown in Table I.

As is clear from the above Table I, in comparison with the core loss of the magnetic core consisting of amorphous alloy thin strip of the same composition, the alloy of this invention, having fine crystal grains, shows excellent soft magnetic properties at high frequencies, high permeability, low core loss after resin moulding and low magnetostriction.

Using a U-function meter, the core loss of magnetic cores of the above alloy composition was also measured, for measurement conditions 100 kHz and 2kG, but using various heat treatment temperatures. The results are shown in Fig. 1. For comparison, the same measurements were performed on a magnetic core of Fe₇₄Cu₂Mo₃Si₉B₁₂, not containing N, manufactured in the same way. These results are also shown in Fig. 1.

It was found that, by introduction of N, the temperature range of heat treatment with which low core loss was obtained with the alloy of this invention was increased.

With alloys according to this invention, Fe-based soft iron alloy can be provided having excellent soft magnetic properties, having fine crystal grains in the desired alloy composition, with high saturated magnetic flux density in the high frequency region, and the required Fe-based soft magnetic materials can be easily manufactured, owing to the wide temperature range of heat treatment possible.

## Claims

1. An Fe-based soft magnetic alloy having fine crystal grains defined by formula (I)
Fe_{100-a-b-c-d}MₐM'_{b}Z_{c}N_{d} (I)
wherein M is at least one element from the following:
Cu, Ag, Au, Zn, Sn, Pb, Sb, and Bi;
M' is at least one element from the following:
Ti, Zr, Hf, V, Nb, Ta, Cr, Mo, W, Mn, Co, Ni, and Al;
Z is at least one element from the following:
Si, P, and B;
and wherein a, b, c, and d expressed in atomic % are as follows:
0.01 ≦ a ≦ 5
0.1 ≦ b ≦ 10
15 ≦ c ≦ 28
0 < d ≦ 8,
and the area ratio of said fine crystal grains in the range of 5 to 30 nm (50 Å to 300 Å) is at least 30%.

2. Alloy according to claim 1, wherein at least 80% of said fine crystal grains are in the range of 5 to 30 nm (50 Å to 300 Å).

3. Alloy according to claim 1 or 2 wherein a is 0.5 to 3 Atomic %.

4. Alloy according to any preceding claim wherein b is 1 to 7 Atomic %.

5. Alloy according to claim 4 wherein b is 1.5 to 5 Atomic %.

6. Alloy according to any preceding claim wherein c is 18 to 26 Atomic %.

7. Alloy according to any preceding claim wherein the ratio of Si/B and/or the ratio Si/P is more than one.

8. Alloy according to any preceding claim wherein d is less than 6 Atomic %.

9. Alloy according to claim 8, wherein d is less than 4 atomic %.

10. A method of treating an Fe-based soft magnetic alloy according to any preceding claim which comprises heat treating said alloy for from one minute to ten hours at a temperature of from 50C° below to 120C° above the crystallisation temperature of said alloy, to segregate the fine crystal grains, the heat treatment preferably being carried out for from ten minutes to five hours.

## Patentansprüche

1. Weiche, magnetische Legierung auf Fe-Basis mit feinen Kristallkörnern, die durch die Formel (I) definiert ist:
Fe_{100-a-b-c-d}MₐM'_{b}Z_{c}N_{d} (I)
wobei M mindestens ein Element von den folgenden ist:
Cu, Ag, Au, Zn, Sn, Pb, Sb, und Bi;
wobei M' mindestens ein Element aus den folgenden ist:
Ti, Zr, Hf, V, Nb, Ta, Cr, Mo, W, Mn, Co, Ni, und Al;
Z mindestens ein Element aus den folgenden ist:
Si, Pb und B;
und wobei a, b, c und d in Atomprozenten ausgedrückt folgendermaßen sind:
0,01 ≦ a ≦ 5
0,1 ≦ b ≦ 10
15 ≦ c ≦ 28
0 < d ≦ 8
und das Gebietsverhältnis der feinen Kristallkörner im Bereich von 5 bis 30 nm (50 Å bis 300 Å) mindestens 30% ist.

2. Legierung nach Anspruch 1, wobei mindestens 80% der feinen Kristallkörner im Bereich von 5 bis 30 nm (50 Å bis 300 Å) liegen.

3. Legierung nach Anspruch 1 oder 2, wobei a = 0,5 bis 3 Atomprozent ist.

4. Legierung nach einem der vorhergehenden Ansprüche, wobei b = 1 bis 7 Atomprozent ist.

5. Legierung nach Anspruch 4, wobei b = 1,5 bis 5 Atomprozent ist.

6. Legierung nach einem der vorhergehenden Ansprüche, wobei c = 18 bis 26 Atomprozent ist.

7. Legierung nach einem der vorhergehenden Ansprüche, wobei das Verhältnis von Si/B und/oder das Verhältnis von Si/P mehr als 1 ist.

8. Legierung nach einem der vorhergehenden Ansprüche, wobei d kleiner als 6 Atomprozent ist.

9. Legierung nach Anspruch 8, wobei d kleiner als 4 Atomprozent ist.

10. Verfahren zum Behandeln einer weichen, magnetischen Legierung auf Fe-Basis nach einem der vorhergehenden Ansprüche, welches die Wärmebehandlung der Legierung über eine Zeit von einer Minute bis zu zehn Stunden bei einer Temperatur von 50°C unter der Kristallisationstemperatur bis 120°C über der Kristallisationstemperatur der Legierung umfaßt, um die feinen Kristallkörner zu trennen, wobei die Wärmebehandlung vorzugsweise über zehn Minuten bis fünf Stunden durchgeführt wird.

## Revendications

1. Alliage magnétique doux ou mou à base de Fe ayant de fins grains de cristal, défini par la formule (I) suivante :
Fe_{100-a-b-c-d}MₐM'_{b}Z_{c}N_{d}
dans laquelle M désigne l'un au moins des éléments suivants :
Cu, Ag, Au, Zn, Sn, Pb, Sb et Bi
M' étant l'un, au moins, des éléments suivants :
Ti, Zr, Hf, V, Nb, Ta, Cr, Mo, W, Mn, Co, Ni et Al
Z étant l'un, au moins, des éléments suivants :
Si, P et B
et où a, b, c, qui sont exprimés en % atomiques, sont l'un des éléments suivants :
0,01 ≦ a ≦ 5
0,1 ≦ b ≦ 10
15 ≦ c ≦ 28
0 ≦ d ≦ 8
et le rapport de l'air desdits fins grains de cristal dont la granulométrie est comprise entre 5 à 30nm (50 Å à 300 Å) est, au moins, de 30%.

2. Alliage selon la revendication 1, caractérisé en ce que 80%, au moins, les dimensions desdits fins grains de cristal sont comprises entre 5 et 30 nm (50Å à 300Å).

3. Alliage selon la revendication 1 ou 2, caractérisé en ce que a est compris entre 0,5 et 3% atomiques.

4. Alliage selon l'une quelconque des revendications précédentes, caractérisé en ce que b représente entre 1 et 7% atomiques.

5. Alliage selon la revendication 4, caractérisé en ce que b est compris entre 1,5 et 5% atomiques.

6. Alliage selon l'une quelconque des revendications précédentes, caractérisé en ce que C est compris entre 18 et 26% atomiques.

7. Alliage selon l'une quelconque des revendications précédentes, caractérisé en ce que le rapport Si/b et/ou le rapport Si/P est supérieur à l'unité.

8. Alliage selon l'une quelconque des revendications précédentes, caractérisé en ce que d est inférieure à 6% atomiques.

9. Alliage selon la revendication 8, caractérisé en ce que d est inférieur à 4% atomiques.

10. Procédé pour traiter un alliage magnétique tendre ou mou à base de Fe, selon l'une quelconque des revendications précédentes, qui consiste à traiter par la chaleur ledit alliage, pendant une période comprise entre une minute et dix heures, à une température entre 50°C et moins de 120°C au-dessus de la température de cristallisation dudit alliage, à séparer les fins grains de cristal, le traitement par la chaleur s'effectuant, de préférence, pendant un temps compris entre dix minutes et cinq heures.
